

# United States Patent

Mauter et al.

[15] 3,650,677

[45] Mar. 21, 1972

## [54] SEA CHEST PROTECTION PROCESS

[72] Inventors: David J. Mauter, Edgewater, N.J.; Jack A. Antinori, Bayside, Long Island, N.Y.

[73] Assignee: Drew Chemical Corporation, New York, N.Y.

[22] Filed: Sept. 25, 1969

[21] Appl. No.: 861,045

[52] U.S. Cl. .... 21/2.5, 21/2.7, 114/0.5 R,  
137/15

[51] Int. Cl. .... C23f 11/10

[58] Field of Search..... 114/0.5 R; 21/2, 7, 2.5;  
137/15; 252/72

[56]

## References Cited

### UNITED STATES PATENTS

|           |         |                     |           |
|-----------|---------|---------------------|-----------|
| 2,450,070 | 9/1948  | Wright.....         | 114/0.5   |
| 2,785,078 | 3/1957  | Keating et al. .... | 21/2.7 UX |
| 2,856,299 | 10/1958 | Westlund .....      | 21/2.7 UX |
| 3,084,791 | 4/1963  | Hawley .....        | 21/2.5 X  |

Primary Examiner—Morris O. Wolk

Assistant Examiner—Barry S. Richman

Attorney—Douglas W. Wyatt

[57]

## ABSTRACT

Method of protecting sea chests of vessels during layup by filling the chest with a substantially biodegradable vegetable oil based composition which has a melting point of between 25° and 50° C.

5 Claims, 2 Drawing Figures



Patented March 21, 1972

3,650,677



FIG. 1



FIG. 2

INVENTORS  
JACK A. ANTINORI  
and  
DAVID J. MAUTER

BY

MARK C. JACOBS  
ATTORNEY

## SEA CHEST PROTECTION PROCESS

This application relates to "sea chests" and to the protection thereof from corrosion. More particularly, it relates to the prevention of fracture of the sea chest's metallic surfaces and the sea valves, and to a filler composition for the sea chests, said filler composition to be utilized during the period of layup for the vessel.

A sea chest may be defined as a conduit fitting open to the sea, secured to the ship or as a part thereof and connected to a piping system of the ship for the purpose of admitting water from the body of water wherein the vessel is situated, to the piping system.

This admission of water can take place for any of several purposes. These include ballasting of the ship as well as for the cooling of systems and for fire fighting.

Each winter on the Great Lakes of the United States and perhaps in certain other area of extreme cold, vessels traversing these waters are laid up due to the inability to navigate the frozen waters. From an engineering viewpoint, it is essential that any equipment that contains water be drained and kept free from water during the so-called layup period until the following spring. Due to the fact that very few drydocks are available in these areas, most of the vessels are laid up in the water.

While inlet and outlet valves on all systems which utilize water either as a coolant or for ballast can be closed and the lines and equipment inboard therefrom can be drained, such is not the case for the sea chests of the vessel.

Essentially, a sea chest can best be described, as previously indicated, as a void space or box on the "skin" of the ship below the water line and which provides a relatively stagnant area at the inlet to a piping system. Reference is made to FIGS. 1 and 2 of the drawing, which will be described in more particularity hereinafter. By providing this stagnant area, free from the currents and pressures created by the momentum of the ship as it moves through the water, the centrifugal pumps which force water into the several systems of the ship are able to maintain suction.

If the sea chest or water inlet boxes are not protected from the ingress of water during the layup period, water would enter the area up to the injection valve, and would, as the temperature dropped, freeze, expand and cause the cracking of and destruction to expensive equipment.

A variety of methods have been tried over the past 50 years to prevent this from occurring and the one which has proven to be most successful is the introduction of a grease-like substance to the sea chest. The most common type of "filler" is a petroleum base product put out by the major oil companies. These products are dark in color, have the consistency of a very heavy grease, do not freeze, and have sufficient resiliency to "give" under the pressure of external ice conditions. However, these are today considered to be unacceptable, as these grease-like substances, when pumped out from the sea chest into the sea, lake, etc., foul and pollute the water due to their lack of biodegradability.

Such pollution problems especially of the Great Lakes, and its beaches, are of grave concern to the states situated on the Great Lakes and to the U.S. Government as well, since these governmental bodies are trying to rehabilitate the beaches, aquatic life, and bird life native to area.

A few years ago, a product which comprised paraffin blended with mineral oil was put on the market as a sea chest filler composition. While the pollution problem was lowered by the use of such compositions, the compositions are not readily accepted by the trade due to their poor handling characteristics, such as minimum resiliency. The heat conductancy of paraffin is such that the entire mass cannot be melted. Rather, like a candle, only the unit volume immediately exposed to heat will soften. For this reason, it is difficult to remove these materials from the sea chest in the Spring. The color of such paraffin based compositions is generally yellow-white and is not esthetic to the eye of the viewer.

It is an object of this invention, therefore, to prepare a biodegradable sea chest filler composition, which possesses good physical process characteristics, and to the composition derived from such process.

5 Another object is the preparation of a sea chest filler composition which is easy to handle during both the filling and pumping out operations.

Still another object is the development of a composition for filling a sea chest which when inserted will prevent the admission of water therein, which composition is biodegradable and has good physical characteristics.

Yet another object is the preparation of a biodegradable, sea chest filler composition of good handling characteristics.

15 A further object is the development of a novel method of preventing corrosion of sea chests during layup.

A still further object is the method of introduction and removal from sea chests and adjoining appurtenant piping of a filler composition which has a wide range of compatibility with other filler materials.

20 An additional object is the provision of a process for the introduction of a filler composition to a sea chest, and for the subsequent removal thereof.

A yet further object is the presentation of a novel method 25 for the prevention of fracture and corrosion of sea chests during periods of vessel layup.

Further objects of the invention will in part be obvious and will in part appear hereinafter.

The invention accordingly comprises the processes involving 30 the several steps and the relation and order of one or more of such steps with respect to each of the others and the product possessing the features, properties and the relation of elements which are exemplified in the following detailed disclosure, and the scope of the application of which will be indicated in the claims.

35 For a fuller understanding of the nature and objects of the invention, reference should be had to the following detailed description, taken in connection with the accompanying drawings, wherein:

40 FIGURES 1 and 2 are partial cross-sectional views at different cross sections of a vessel, and are intended to depict that area of a vessel wherein a sea chest is to be found. As such, sea water injection and pipe opening, 13, and valve fitting, 10, are found only in FIG. 1, which is a further aft cross section. In the more forward cross section, the strainers, 22, and retainer, 21, are shown. The sea chest is shown to comprise a top 11, a side 20, a bottom 14, two end plates, one of which is shown, 18, and a curved side consisting of hull, 17, in 45 which are found two strainers, 22, whose front or inlet portion is not shown.

45 The pipe retainer 12, and pipe 16 are intended to hold the pipe that terminates at 13, in place. The valve fittings 10 are used to provide access for the filler to the sea chest at layup and for steamlines or other means for removal thereof at fit-out time.

50 During the operation of the vessel, water needed for ship functions enters the sea chest area through the strainers, which are open to the sea, and the water is pumped to the various facilities such as the condensers, ballast tanks or the evaporators, through a pipe opening such as 13. At layup time, the sea chest filler composition is pumped in through valves 10, and allowed to solidify. The screen or holes in the strainer, 55 22, help keep the solidified material in place. At spring thaw, or when the ship is to be put into service, steam or other heated liquid or gas is pumped in through the valves 10, into the sea chest to melt the filler composition, which then floats out through the strainers 22, and into the surrounding water 60 19.

65 In short, the objects of this invention are accomplished by utilizing a vegetable oil based composition as a sea chest filler composition. A preferred vegetable oil based composition is prepared from still bottom residues derived from the distillation 70 of fatty acids from the various vegetable oils.

Specifically, when vegetable oils such as coconut oil, palm oil, soybean, cottonseed oil, corn oil and the like are distilled to prepare fatty acids, grease-like still residues remain. These are separated away from the oils. The oils, residues, and fatty acids may each in turn be treated as per techniques, briefly discussed infra, which are known to those dealing in fats and oil chemistry, to yield compositions that are the filler compositions of this invention. These compositions possess physical characteristics of a nature, which render them suitable as sea chest filler compositions and handling characteristics which makes them easy to handle during both the filling and pumping out operations of the sea chest.

It is known to those skilled in the art that fatty acids can be prepared by the treatment of vegetable oils by techniques known as refining and saponification. Fatty acids can also be prepared by the process known as fat splitting or fat hydrolysis of mixed triglycerides, which themselves are obtained from vegetable oils. Refining, saponification and fat splitting are well known techniques and are discussed at length in such references as Bailey's Industrial Oil and Fat Products, 3rd Edition (c) 1964.

Specifically, when vegetable oils such as coconut, palm, soybean, peanut, cottonseed, corn, palm kernel, sunflower and the like, as well as the hydrogenated and/or rearranged forms of said vegetable oils, are treated to yield free fatty acids and glycerine, grease-like still residues remain as a by-product of these processes. These grease-like still residues are collected and comprise one source of the filler compositions suitable for this invention. As can be appreciated these "still residues" will vary widely in their percentage compositional makeup and their chemical composition, in view of the fact that the actual composition is a function of the type of vegetable oil being treated and the extent to which the fatty acid recovery process has been carried out. It is seen, therefore, that the ingredients of such still residues based upon any particular oil will be substantially the same. For instance, it has been reported that crude cottonseed oil prior to treatment contains such constituents as raffinose, pentosans, resins, peptones, inositol phosphates, chlorophyll, fatty acids and several other components.

It is to be noted that the term "vegetable oil" is seen to encompass not only the oil per se, but also hydrogenated, and/or rearranged oils which likewise will yield, upon treatment, the still residues utilized in this invention as filler compositions.

Similarly, when vegetable oils are saponified; i.e., treated with caustic soda or potassium hydroxide to prepare soap stock, the residues that remain after collection of the soap stock, comprise another source of filler compositions utilizeable for the process of this invention.

It is to be seen that this prime soap stock can also be utilized as a source of filler composition, but it is too costly to utilize it as such.

The filler compositions can also be prepared by the process of splitting refined oils. In this process, triglycerides are reacted with water under heat and pressure to yield glycerol and a mixture of free fatty acids. The mixture of acids is then separated from the glycerol by neutralization techniques known in the art. The mixture of acids, now without glycerol, is acidified and fractionally distilled. The remaining material after the fractional distillation is retreated with a base such as monoethanolamine, diethanolamine, calcium carbonate, magnesium hydroxide, lithium hydroxide and the like, to yield a low grade soap stock. This low grade soap stock is collected and comprises a third source of filler compositions for this invention.

It is to be understood that the crude fatty acid mixture with glycerol, as well as the fatty acid mixture after separation from the glycerol, can also be utilized as the filler composition of this invention, but it is economically unfeasible to do so.

In summary, it is seen that vegetable oil based filler composition should have a pH of about 7, a high flash point of about 226° C. C.O.C., a melting point range of about 25° C. to about 50° C., preferably 30° to 40° C., and be a non-crystalline solid with a low coefficient of expansion and high resiliency.

The usual method for inserting sea chest filler compositions is to melt the composition and to pump it into the chest according to known maritime techniques. This process will be described in more detail below.

5 The usual method of cleaning the sea chest is to attach a steam line to the valve of the sea chest and melt the filler composition followed by a conventional pumping out step. Paraffin-mineral oil based compositions do not transfer heat such that the total body of filler composition is melted. Rather, the entering steam melts a hole in the composition at the point of initial contact, but that portion of the composition distant from the valve remains intactly solid. This phenomenon necessitates the use of large quantities of steam, and an excessive amount of time to accomplish removal of the composition 10 from the sea chest. While biodegradable, they are dangerous to fish, wild life and humans on ingestion.

15 The filler compositions of this invention on the other hand, melt readily between 80°-90° F. and are thus easily pumped into the sea chest. Furthermore, they melt completely during the application of heat, as from a steam line and can thus be 20 easily removed by a pumping operation.

25 The compositions of this invention readily adhere to the metallic surfaces of the valves, piping, etc., thus preventing corrosion thereof and solidify within the sea chest at temperatures below about 80° F., and are seen, therefore, to be excellent sea chest filler compositions. In addition these compositions are completely biodegradable, and non poisonous to fish and wildlife on ingestion. This last factor is quite an important 30 property of these compositions of this invention, for it is known that certain chemical compositions, such as those derived from petroleum while not dangerous to the feathers and other external surface of birds will kill the birds when they ingest such compositions during attempts to remove the compositions from their bodies.

35 As to the use of the filler composition, it should be pumped directly into the sea chest at layup time to force the water out of the sea chest and to prevent ingress of water and/or ice during the layup period. This is accomplished by removing the 40 head of the steel drum, which is a typical shipping container for such compositions and inserting a steam coil into the filler until the composition melts at about 80° to 90° F., and then pumping it into the sea chest by way of a small hand pump connected to fill lines. Naturally, the amount of filler required 45 for a particular sea chest will vary with the size of the sea chest. To facilitate removal of the filler during the "fit-out" period in the Spring, steam lines are attached to valves on the sea chest to melt the filler which is then "blown overboard" by 50 the steam pressure (usually 5 to 10 p.s.i.g.). In actual fact, once the filler starts to melt, it has a tendency to virtually slide out of the sea chest.

55 While the above described procedures can be readily accomplished without a large expenditure of funds, it is to be readily appreciated that the filler can be inserted into and withdrawn from the sea chest and its appurtenant piping by the use of more sophisticated machinery. Thus any positive displacement pump can be used as the mode of transmission, and any heat source capable of melting the filler composition 60 can be utilized. Persons of the marine industry would be well aware of the existence of these alternate pieces of apparatus to accomplish the desired results.

65 The invention will be illustrated in greater detail in conjunction with the following specific examples which, however, are not to be limited to the details set forth therein and are intended to be illustrative only.

#### EXAMPLE I

70 Into the sea chest of a Great Lakes steamer about 500 pounds of a melted filler composition comprising soap stock derived from the splitting and subsequent neutralization of soya bean oil are pumped in, over a period of about 30 minutes, with several minute pauses between pumping intervals, to allow for solidification and compaction of the filler.

## EXAMPLE II

Approximately, 1,100 pounds of a filler composition derived from the refining of coconut oil, and which exists as a grease-like substance are delivered to ship side. At an atmosphere temperature of about 0° F., the filler is melted to a liquid by immersing a heating element therein. 500 pounds of fluid filler composition are then pumped into the sea chest of a Great Lakes Steamer, type Ore Boat by use of a small positive displacement pump. After a pause in the pumping operation to allow for solidification of the filler, pumping is resumed. Additional filler as required is pumped into the sea chest until the chest is completely occupied by filler composition.

In order to determine the order of magnitude of a vegetable oil based filler composition and biodegradability, a typical sample was submitted to a leading Eastern testing company to determine the Biochemical Oxygen Demand (B.O.D.) for such product. It was found that the B.O.D. of the samples was 300,000 p.p.m., which fact means that there was a high level of biochemical oxygen consumption which is coincident with biochemical degradation. It is believed that other samples would have a B.O.D. approaching or better than 300,000 p.p.m. The B.O.D. test is a well known method for determining biodegradability and is reported in "Standard Methods for the Examination of Water and Waste Water," published by the American Public Health Association, 12th Edition 1965, p. 524.

Since certain changes may be made in the above products, compositions and processed without departing from the scope

of the invention herein involved, it is intended that all matter contained in the above description shall be interpreted as illustrative and not in a limiting sense.

We claim:

- 5 1. A process for preventing fracture of a vessel's sea chest during periods of cold weather layup of said vessel, which comprises filling the sea chest with a substantially biodegradable vegetable oil based filler composition having a melting point range of about 25° C. to about 50° C.
- 10 2. The process of claim 1 wherein said filler composition is soya bean oil based.
- 15 3. The method of preventing fracture and corrosion of a ship's sea chest without subsequent pollution of the water which comprises using as the sea chest filler composition, a vegetable oil based substantially biodegradable filler composition having a melting point range of about 25° C. to about 50° C.
- 20 4. The method of claim 3 wherein the composition is coconut oil based.
- 25 5. The process of preventing fracture in a sea chest during layup without subsequently polluting the water which comprises melting a vegetable oil based substantially biodegradable filler composition, having a melting point of from about 25° C. to about 50° C., pumping said filler composition into the sea chest, at the beginning of the vessel layup period and the end thereof, melting said filler composition, and allowing it to dissipate into the surrounding water.

\* \* \* \* \*

30

35

40

45

50

55

60

65

70

75